

H. C. HARRISON.

CRYSTALLINE FERROSILICON PRODUCT AND METHOD OF MAKING THE SAME.

APPLICATION FILED JULY 30, 1909. RENEWED SEPT. 1, 1914.

1,134,127.

Patented Apr. 6, 1915.



Witnesses

Byron Collings.

Jas. E. Dodge.

Inventor

H. C. Harrison by  
Wickson, Fisher &  
Witherspoon, Attorneys.

# UNITED STATES PATENT OFFICE.

HERBERT CHAMPION HARRISON, OF LOCKPORT, NEW YORK, ASSIGNOR, BY MESNE ASSIGNMENTS, TO ELECTRO METALLURGICAL COMPANY, A CORPORATION OF WEST VIRGINIA.

## CRYSTALLINE FERROSILICON PRODUCT AND METHOD OF MAKING THE SAME.

1,134,127.

Specification of Letters Patent.

Patented Apr. 6, 1915.

Application filed July 30, 1909, Serial No. 510,477.

Renewed September 1, 1914. Serial No. 859,721.

To all whom it may concern:

Be it known that I, HERBERT CHAMPION HARRISON, a subject of the King of Great Britain, residing at Lockport, in the county 5 of Niagara and State of New York, have invented certain new and useful Improvements in Crystalline Ferrosilicon Products and Methods of Making the Same; and I do hereby declare the following to be a full, 10 clear, and exact description of the invention, such as will enable others skilled in the art to which it appertains to make and use the same.

This invention relates to crystalline ferro-silicon products and methods of producing 15 the same, and has for its object to produce such a product in a crystalline form which will correspond substantially to the formula  $Fe_3Si_7$ , or to 54.2 per cent. silicon.

With these objects in view the invention 20 consists in the novel method and product hereinafter more fully disclosed and particularly pointed out in the claims.

Referring to the drawing forming a part 25 of this specification, in which the figure illustrates a conventional form of an electric furnace suitable for carrying out the process, and for producing the product: 1 represents the suitable electrodes, 2 the furnace, 3 the 30 charge, and 4 the molten product.

In carrying out the method, the ferro-silicon charge is so proportioned that there will be produced a ferro-silicon alloy containing as nearly as possible between 53 and 35 54.5 per cent. of silicon. The same is heated in the furnace in the usual way, is tapped out and cooled and then broken up, when throughout the product are found matrices filled with bright, shining, hard, brittle crystals in a plate form which analyze about 54.2 per cent. silicon, depending upon whether the 40 particular matrix selected is relatively rich or poor in silicon. If the matrices are melted and permitted to cool, these crystals 45 invariably solidify first, which tends to show that they have a higher melting point than the ferro-silicon alloys on either side of the same. Crystals from the poorer matrices probably contain about .7 per cent. of impurities, while crystals from rich matrices 50 analyze practically 54.2 per cent. silicon, corresponding to the formula  $Fe_3Si_7$ , taking the atomic weight of iron as 55.9, and of silicon as 28.4. These crystals are, of course, a

much purer compound of iron and silicon 55 than the usual commercial alloys, and, therefore, they offer special advantages in metallurgy, over the regular alloys of say, 25 to 60 per cent. silicon. They contain less carbon and phosphorous than do such alloys, and 60 having a slightly higher melting point than the impurer alloys they are less likely to lose their silicon during the process of purifying the metal. In other words, it is well recognized in metallurgy, that it is very important 65 to obtain the purest product possible, and it is obvious that a crystalline product of this nature is purer than the chance alloys heretofore employed. It is also probable that when the silicon is liberated from a chemical 70 compound, as is the case here, it being in a nascent state, so to speak, that it will be more active chemically in the molten iron than would be the case were it merely liberated 75 from an alloy.

In many cases the crystals need not be separated from their matrices before being used, for the mixture consisting of the crystals and matrices can always be depended on to analyze substantially between 53 and 54.5 80 per cent. of silicon, which is a product sufficiently pure for many purposes. If the charge is made up so as to produce other than 53 to 54.5 per cent. of silicon the crystal product becomes less, and it can be made to 85 so widely differ from this silicon content that the crystal product will disappear entirely. In some cases the matrices on either side of the crystals are found to contain only 90 about 51.28% of silicon.

### What I claim is:

1. The method of producing crystalline ferro-silicon corresponding to the formula  $Fe_3Si_7$ , which consists in so chemically proportioning a ferro-silicon furnace charge as 95 to produce substantially between 53 and 54.5 per cent. of silicon; and in suitably producing ferro-silicon from said charge in an electric furnace by maintaining the temperature at or above a predetermined critical 100 temperature, substantially as described.

2. The method of producing crystalline ferro-silicon corresponding to the formula  $Fe_3Si_7$ , which consists in so chemically proportioning a ferro-silicon furnace charge as 105 to produce substantially between 53 and 54.5 per cent. of silicon; in suitably producing ferro-silicon from said charge in an electric

- furnace by maintaining a constant temperature above a critical temperature; and in separating out the crystals thus formed, substantially as described.
- 5 3. The herein described ferro-silicon product consisting of matrices of ferro-silicon containing substantially between 53 and 54.5 per cent. of silicon and charged with ferro-silicon crystals corresponding to the formula
- 10  $\text{Fe}_3\text{Si}_7$ ; substantially as described.
4. The herein described ferro-silicon product consisting of bright, hard, brittle, plate like, crystals corresponding to the formula  $\text{Fe}_3\text{Si}_7$ ; substantially as described.

In testimony whereof, I affix my signature, in presence of two witnesses.

HERBERT CHAMPION HARRISON.

Witnesses:

W. R. CULMER,  
N. GOULD ALLEN